

## UNITED STATES PATENT OFFICE

1,967,740

## METHOD OF MANUFACTURING MOLDS

Eugen Brill, Berlin, Germany, assignor to the firm of Schering-Kahlbaum, A.-G., Berlin, Germany, a joint-stock company of Germany

No Drawing. Application January 31, 1931, Serial No. 512,739. In Germany April 3, 1930

## 1 Claim. (Cl. 18—48)

My invention relates to improvements in the method of manufacturing objects from porcelain or cast metal and in the mold used in the said method, and more particularly in the method used for example in the manufacture of fillings for teeth in which the plug is made by means of a mold shaped according to the cavity of the tooth. In the manufacture of such plugs it is necessary to coat the mold with a thin metal foil ordinarily made from a noble metal such as platinum or gold, in order to prevent baking together of the plug and the mold when burning or casting the material. The object of the improvements is to provide a method by means of which the said coating may be applied in a most simple way, and in which the said coating is exceedingly thin and dense, and with this object in view my invention consists in applying the coating in colloidal form and together with a carrier thereof.

For the purpose of explaining the invention more in detail several examples embodying the same will now be described.

In accordance with my invention I add the metal in colloidal solutions to the material from which the mold is manufactured, I manufacture the mold from the said material, and I heat the mold either before or after putting the porcelain or metal from which the plug is made into the same. By thus heating the mold a very thin and dense metal coating is produced. The method is important not only in the manufacture of objects from porcelain by molding, but also in the manufacture of complicated objects of metal such as tooth plugs made from metal. In the manu-

facture of such plugs the metal may be immediately cast into the mold in which the cavity is not provided with a metal coating because the cast metal does not adhere to the mold. However if a coating is not used it happens that 30 minute air bubbles are left between the walls of the mold and the material cast into the same which produce irregularities on the surface of the metal casting. When coating the mold in the manner described above by means of a colloidal 35 metal solution this objection is obviated, and it is possible to manufacture exact tooth plugs or other pieces of metal of very complicated shape by casting the metal into a mold which before has been coated by colloidal metal.

While in describing the invention reference has been made to particular examples embodying the same I wish it to be understood that my invention is not limited to the methods of applying the coating of colloidal metal described herein, and 75 that various changes may be made in the said method without departing from the invention.

## I claim:

The herein described method of manufacturing molds for making porcelain fillings for teeth, consisting in applying a colloidal metal solution by adding the same to the basic mass from which the mold is made, making an imprint, and heating the mold after the imprint, thereby causing evaporation of the solution agent of said colloidal 80 metal solution, so that a colloidal metal coating 85 forms on the surface of the mold.

EUGEN BRILL.

35

90

40

95

45

100

50

105

55

110